

## UNITED STATES PATENT OFFICE

1,997,316

MOISTURE RESISTANT FILAMENTS OF  
CELLULOSE ACETATE

Paul C. Seel, Rochester, N. Y., assignor to Eastman Kodak Company, Rochester, N. Y., a corporation of New York

No Drawing. Application December 24, 1929,  
Serial No. 416,286

6 Claims. (Cl. 106—40)

This invention relates to artificial filaments for textile and other purposes and particularly such filaments which have been prepared from cellulose acetate having high moisture resistance.

Since the time of Chardonnet and his original artificial silk made of nitrated cellulose which was regenerated prior to weaving, it has been the desire of investigators in this art to produce artificial silk filaments which would have high strength, whether in the wet or dry state. Attempts to increase the wet strength of such filaments have resulted in their manufacture from dissolved cellulose and from the various types of cellulose esters, for example, the mixed cellulose acetate-nitrate, cellulose propionate, cellulose formate, etc., as well as in the treatment of the formed filaments which may have been manufactured by any of the usual processes, for instance,—the viscose or cuprammonium processes, by the treatment of the filament either with a sizing or other water impervious layer to inhibit this loss of strength while the filament is in the moist condition. In spite of these expedients of sizing coating or impregnating of the filaments or the application of various water-impervious esters of cellulose thereto, the wet strength of the artificial filaments has not been increased to the dry strength of the filament.

I have found that the preparation of artificial filaments from a solution or dope containing a particular type of moisture-resistant cellulose acetate will produce a filament, due to this unexpected resistance to moisture, of exceptional quality. The type of cellulose acetate which I prefer to use is of the acetone-soluble variety, which has been hydrolyzed to a particular degree, thus rendering it exceedingly more resistant to moisture than the usual acetone-soluble cellulose acetate. The acetyl content of such an acetate will run in the neighborhood of from 38% to 42% and may be prepared in any of the following described manners.

Artificial filaments, when prepared from this type of cellulose acetate, have increased wet strength due primarily to their great resistance to moisture. I have found that a solution of this acetate in acetone, with or without the use of the ordinary type of plasticizer such, for instance, as monochlornaphthalene, triphenylphosphate, monoacetin or triacetin or similar plasticizers, will produce such a filament by extrusion into a heated chamber, whereby the volatile solvent is removed and the filament coagulated. The filament may likewise be prepared, if desired, by an extrusion of the dope into a coagulating bath

which removes the volatile solvent contained in the dope and likewise coagulates the same. This bath, if desired, may be composed of a solution of a suitable plasticizer whereby this plasticizer is caused to penetrate into the filament, such a process being described in the copending application of Farrow et al. Serial No. 347,813 filed Mar. 18, 1929.

The cellulose acetate which I have found to have these desirable characteristics may be prepared from any type of cellulose triacetate such as that produced by the usual pretreating and acetylating methods or, for instance, by the process as described in U. S. Patent No. 1,683,347, Harry Le B. Gray and Cyril J. Staud, September 4, 1929. This triacetate of cellulose containing approximately 44.8% acetyl is hydrolyzed either by the addition of acetic acid and water or by the addition of acetic acid, water and a mineral acid catalyst or by the production within the acetylating bath of water which may be effected by the addition of an alcohol or other water former thereto.

The cellulose acetate which I prefer to use is obtained by stopping the hydrolysis of the cellulose acetate when approximately 90% or more of a sample taken from the hydrolyzing solution, precipitates in a mixture of 40% water and 60% acetone by volume when carried out in the manner described below. Cellulose acetate which has been accurately hydrolyzed to this degree has attained exceptional qualities of water resistance and good flexibility which are not shown by any other cellulose acetates which are soluble in acetone. Furthermore, the addition of phenyl or ortho cresyl para toluene sulfonate, triphenyl phosphate or tricresyl phosphate to a cellulose acetate having a precipitation value of 90-97 per cent will increase even further the moisture resistance of the cellulose acetate. Above 97 per cent precipitation value little or no added moisture resistance will be effected by such an addition and any of the usual plasticizers may be employed with this exceedingly high precipitation value acetate to impart the desired plasticity, very slight if any additional moisture resistance being effective by their presence.

In order that the method of determining this particular point in the hydrolysis of the cellulose acetate may be more thoroughly understood the exact method used is here disclosed; A sample of the cellulose acetate which has been removed from the hydrolyzing reaction mixture is dried under standard conditions; to 5.00 grams of this dried cellulose acetate there are added 100.0 cc.

of acetone of 99% or better,—the whole thing stirred until a homogeneous mixture results. The container in which the solution is being effected is closed. To this dope is added slowly from a 5 pipette and with thorough stirring 150.0 cc. of a solution consisting of two parts of distilled water and one part of acetone by volume. Care should be taken to keep the solvents and mixtures at a 10 temperature of  $20^{\circ} \pm 1^{\circ}$  C., wherever volumes are being measured.

At the end of the addition of the acetone-water solution, a mixture is obtained containing 40% water by volume (neglecting contraction), in 15 which is suspended the precipitated cellulose acetate. This is allowed to stand for 12 hours at  $20^{\circ}$  C., and 25 cc. of the clearest supernatant solution are removed with a pipette. At the end of this time, precipitation has reached equilibrium and proceeds no further. This 25 cc. portion 20 is centrifuged in a stoppered bottle at a high speed until the liquid is perfectly clear. Exactly 5 cc. of the liquid are removed with a pipette and evaporated to dryness on a tared watch glass. If  $W$  is the weight of the residue in grams, the 25 "precipitation value" which equals the percent cellulose acetate precipitated will equal

$$= 100 - W \times \frac{250}{5} \times \frac{1}{5} \times 100 \\ = 100 - 1000W$$

I have found that artificial filaments for the preparation of artificial silk or like products, as 30 prepared from a "dope" containing a hydrolyzed cellulose acetate, that gives a precipitation value 35 in the above test of 90% or better, have an exceptionally high water resistance, with its corresponding increase in wet strength, due to this resistance to water. It will be understood that 40 while this cellulose acetate artificial filament may not have an appreciably greater strength when that strength is computed upon the percentage of moisture contained in the filament, nevertheless, by the use of this type of cellulose acetate, when compared to a cellulose acetate filament subjected to equivalent moisture conditions, the wet 45 strength of the filament prepared from my type of cellulose acetate will be decidedly greater. To obtain this desirable product, it is but necessary to control the hydrolysis by the utilization of suitable hydrolyzing baths in which the degree of 50 deacetylation and the precipitation value of the cellulose acetate may be readily and accurately controlled. The method of so controlling this 55 hydrolysis is described in the U. S. Patent No. 1,878,953 of C. J. Malm.

The precipitation value of 90% or more may be obtained by the usual hydrolyzing methods, such as indicated below, providing, of course, that the hydrolysis be stopped at the correct point. 60 When this point has been reached, it is often very difficult instantly to stop further hydrolysis of the cellulose acetate so that the resulting product will not have a precipitation value of less than 90%. Accurate and substantially instantaneous stopping of the hydrolysis may be effected by the process as described in the pending application of C. J. Staud and J. T. Fuess, Serial No. 398,807 (Pat. No. 1,895,351). Other methods of effectively controlling the hydrolysis in order 65 that it may be stopped when the product has the required precipitation value may be employed. The following hydrolyzing processes which I call the "acid final" or "water final" have proved efficient. In the "acid final" type of hydrolysis 70 mineral acids (i. e. hydrochloric or sulfuric acid)

are added with acetic acid and water to the so-called "first stage" cellulose acetate "dope": i. e., the cellulose acetate solution attained at the end of the acetylating step, usually a solution of a fully acetylated cellulose. The quantity of mineral acid added is adjusted so that hydrolysis requires from 30 to 50 hours at a temperature of 95 to  $100^{\circ}$  F. At this temperature, it is somewhat difficult at all times to regulate the exact time at which the hydrolysis should be stopped, as 10 noted above, to give a precipitation value of 90%; at a lower temperature, however, of say  $70^{\circ}$  F., the time of treatment is increased to from 5 to 10 days with the resultant increase in the accuracy of control. 15

Of the two hydrolyzing processes, I prefer, however, to use the "water final" method which I will now describe. This may be carried out by the use of acetic acid and water without the addition thereto of further mineral acid catalysts, 20 as the catalysts from the "first stage" of the acetylation are usually sufficient. At a temperature of  $70^{\circ}$  F., hydrolysis conducted in this manner will require 20 to 25 days to obtain a product having precipitation value of approximately 25 90%; at a temperature of  $90^{\circ}$  to  $100^{\circ}$  F., the time will be reduced to from 8 to 12 days. It is apparent that with the long period of hydrolysis, as here described, and by the use of the process 30 of Staud and Fuess for the stopping of the hydrolysis, accurate deacetylation of the cellulose acetate may thus be obtained. 35

After hydrolysis, the cellulose acetate may be isolated, washed, and dried by any of the usual processes and, after solution in acetone or other suitable solvent, with or without plasticizers, may be extruded in any of the well known methods for the preparation of artificial filaments. Cellulose acetate of this type, therefore, may be prepared from any of the usual acetylating solutions and formed by any of the well known processes into artificial filaments without in any way departing from this invention or sacrificing any of its advantages. 45

In the claims hereunto appended, where reference is made to the "precipitation value" of the cellulose acetate to be employed it will be distinctly understood that such "value" is a physical characteristic of the cellulose acetate which is to be determined in accordance with the method above set forth in detail. The fact that the method of determining the precipitation value should be followed closely is not, of course, to be understood as limiting the scope of the invention since that is limited only by the specified range of the precipitation value of the cellulose acetate to be employed. 50

While my product is primarily filaments of cellulose acetate composed principally of acetone-soluble cellulose acetate having the above described degree of hydrolysis, I have found that other filaments composed of any of the usual types of rayon, such as viscose, coprammonium silk, and denitrated cellulose nitrate, may be rendered more moisture resistant if they be encased in a coating of this type of cellulose acetate. This may be done by passing the rayon in filament form through a bath containing the cellulose acetate in solution. 60 65 70

What I claim as my invention and desire to be secured by Letters Patent of the United States is:

1. Artificial filaments of the rayon type having an unusual degree of resistance to moisture and 75

increased wet strength essentially consisting of an acetone-soluble cellulose acetate having a precipitation value of at least 90%.

2. Artificial filaments of the rayon type having an unusual degree of resistance to moisture and increased wet strength formed from a solution containing acetone-soluble cellulose acetate having a precipitation value of from 90% to 97%.

10 3. An artificial filament of the rayon type having an unusual degree of resistance to moisture and increased wet strength formed from a solution containing acetone-soluble cellulose acetate having a precipitation value of from 90-97%

15 and o-cresyl para toluene sulfonate.

4. Artificial filaments of the rayon type having an unusual degree of resistance to moisture

and increased wet strength formed from a solution containing acetone-soluble cellulose acetate having a precipitation value of from 90% to 97% and triphenyl phosphate.

5 5. Artificial filaments of the rayon type having an unusual degree of resistance to moisture and increased wet strength essentially consisting of acetone-soluble cellulose acetate having a precipitation value of from 90% to 97% and tricresyl phosphate.

10 6. Artificial filaments of the rayon type having an unusual degree of resistance to moisture and increased wet strength, essentially consisting of acetone-soluble cellulose acetate having a precipitation value of from 90% to 97% and a 15 plasticizer.

PAUL C. SEEL.